

1

3,119,705

**INERT SIMULANT FOR EXPLOSIVE**  
Irving L. Kintish, Bronx, N.Y., and John E. Rainier,  
Morris Plains, N.J., assignors to the United States of  
America as represented by the Secretary of the Army  
No Drawing. Filed Mar. 22, 1961, Ser. No. 97,703  
6 Claims. (Cl. 106—220)  
(Granted under Title 35 U.S. Code (1952), sec. 266)

The invention described herein may be manufactured and used by or for the Government of the United States of America for governmental purposes without the payment of any royalties thereon.

The general purpose of this invention relates to new compositions for use as simulant for explosives and based upon the use of the glyceride of 12-hydroxy stearic acid and inert fillers. The compositions simulate the various properties of explosives except the explosive characteristic itself.

In certain circumstances of ammunition development and testing, it has been the general practice to employ actual rounds of explosive to establish various criteria for storage, handling, etc. and to determine the extent to which temperature, humidity, etc. affect the ammunition item. Although the use of actual live ammunition has served such purpose, it leaves something to be desired with regard to the everpresent hazard created by the explosive feature.

Those concerned with the military program of ammunition development and testing have long recognized the need for an inert ammunition simulant. The present invention serves to fulfill this need.

An object of the present invention, therefore, is to provide non-explosive simulants which can be used in the development and testing of all items of ammunition.

A further object of this invention is to provide an explosive simulant which can be used with relative safety for practice and training purposes.

Other objects and advantages of the invention will hereinafter become more fully apparent from the following description and appended claims.

For compositions to be acceptable for use as simulants for explosives, particularly in military applications, they should conform to the following requirements; namely, (1) reproduce the density and physical properties of the specific explosive, (2) remain stable between  $-65^{\circ}$  F. and  $160^{\circ}$  F., be non-hydroscopic, and exhibit no segregation or exude when subjected to storage in this temperature range, (3) should be non-toxic, undergo no adverse reaction when in contact with conventional explosives, nor exhibit any corrosive effects upon contact with metals, (4) in the molten and solidifying phases, during casting, they should possess viscosity and shrinkage characteristics similar to the specific explosive, (5) they should be readily machinable and removable from the ammunition item, as for example, by steam, and (6) in melt-loading, the material should be pourable for a minimum time of eight hours.

Materials such as sand, gravel, oil, sawdust, paraffin, hydrocarbon waxes, sulfur, silica, metallic salts, metal oxides, metals, halogenated waxes, halogenated diphenyls, halogenated diphenyl benzenes, calcined gypsum, perlite, vermiculite, Portland cement, aromatic hydrocarbons, and organic acids, have been used. Although these materials alone or in combination, simulated the density of the specific explosive being replaced and were relatively low in cost, they were deficient in many of the other essential requisites previously referred to.

Accordingly, the present invention is based upon the discovery of formulating with glyceride of 12-hydroxy stearic acid and suitable fillers a novel group of non-explosive inert materials which more closely simulate the

2

specific explosives than any of the heretofore known compositions.

The new compositions broadly described above are best illustrated by the following examples:

#### Example I

For the preparation of a composition simulating Composition B (density 1.65) for cast loading, 30 parts by weight of glycerine of 12-hydroxy stearic acid and 5 parts by weight of wood rosin are placed in a steam jacketed kettle equipped with an agitator. The ingredients are melted at about  $100^{\circ}$  C. and when molten, 65 parts by weight of dead burned gypsum are slowly added with constant agitation until a homogeneous mixture is obtained. Items of ammunition may be loaded directly with this molten mixture or, alternatively, may be cast into a predetermined shape and subsequently loaded. Mixes of this composition have been maintained for 5 days at  $110^{\circ}$  C. while others have been allowed to solidify and then remelted and in neither instance was there any adverse effect or detectable change.

Paraffin and other hydrocarbon waxes as well as halogenated hydrocarbon waxes may be substituted for the wood rosin.

#### Example II

For the preparation of a composition simulating TNT for press loading, 40 parts by weight of glyceride of 12-hydroxy stearic acid and 60 parts by weight of dead burned gypsum are dry blended to a uniform mixture. Items of ammunition are loaded by placing increments of the resultant mixture, unheated, into the item and applying the desired pressures and dwell time.

TNT simulants for press loading generally are adjusted to density values of TNT compositions, i.e., between 1.34 and 1.60. The resulting compositions meet all the essential requirements for acceptable explosive simulants and thereby permit the use of the same techniques and equipment to case or pressload into carriers as used with the explosives themselves.

Although dead burned gypsum has been used as the major filler in the above examples, such other fillers as sawdust, cork, pumice, perlite, salts, starches, resins, vermiculite, metal oxides, metals, waxes, oils, other glycerides, and lecithin as well as other suitable materials may be employed to adjust the density of the resulting composition to any desired value. Suitably inert metals and metallic oxides are those found naturally occurring, i.e., as minerals.

What is claimed and desired to be secured by Letters Patent of the United States is:

1. An inert composition simulating a solid explosive, consisting essentially of about 30 to about 40 parts by weight of the glyceride of 12-hydroxy stearic acid, about 60 to about 65 parts by weight of dead burned gypsum, and 0 to about 5 parts by weight of wood rosin, said composition having a density substantially corresponding to that of said explosive.

2. An inert composition simulating TNT, consisting essentially of the glyceride of 12-hydroxy stearic acid and a filler selected from the group consisting of cement, gypsum, minerals composed of siliceous materials, metallic oxides, and metals in the free state, the said filler being added in amounts sufficient to provide the said composition with a predetermined density substantially corresponding to the density of TNT.

3. A method for producing an inert composition simulating Composition B, which comprises the steps of mixing about 30 parts by weight of the glyceride of 12-hydroxy stearic acid and about 5 parts by weight of wood rosin, melting the mixture, heating the resulting melt to a temperature of about  $100^{\circ}$  C. and maintaining this tempera-

ture while adding thereto about 65 parts by weight of dead burned gypsum, homogenizing the said gypsum in the said melt, and lastly, cooling.

4. A method for producing an inert simulant for a solid explosive composition which comprises the steps of mixing about 6 parts by weight of the glyceride of 12-hydroxy stearic acid and about 1 part by weight of an additive selected from the group consisting of wood rosin, hydrocarbon waxes, and halogenated hydrocarbon waxes, melting the mixture, heating the resulting melt to a temperature between about 100 and 110° C., and maintaining this temperature while adding thereto a filler selected from the group consisting of cement, gypsum, minerals composed of siliceous materials, metallic oxides, and metals in the free state, the said filler being added in an amount sufficient to provide the said composition with a density substantially equivalent to that of said explosive composition, homogenizing the said filler in the said melt, and lastly, cooling.

5. In the manufacture of explosive materials including

10

15

20

the pretesting operations of casting, machining, and press loading, the improvement which comprises the step of employing in the said testing operations instead of the said explosive, an inert simulant comprising 12-hydroxy stearate and a filler selected from the group consisting of cement, gypsum, minerals composed of siliceous materials, metallic oxides, and metals in the free state, the said fillers being added in an amount to provide the resulting composition with a density equivalent to that of the said explosive.

6. The method according to claim 12 in which the said filler is dead burned gypsum.

References Cited in the file of this patent

UNITED STATES PATENTS

|           |             |       |               |
|-----------|-------------|-------|---------------|
| 1,276,508 | Ellis       | ----- | Aug. 20, 1918 |
| 1,987,553 | Fisher      | ----- | Jan. 8, 1935  |
| 2,077,094 | Byers       | ----- | Apr. 13, 1937 |
| 2,251,225 | Dangelmajer | ----- | July 29, 1941 |
| 2,266,810 | Ruben       | ----- | Dec. 23, 1941 |